

## UNITED STATES PATENT OFFICE.

HARRIETT B. DEVLAN, OF JERSEY CITY, NEW JERSEY.

## ANTI-FRICTION COMPOUND.

SPECIFICATION forming part of Letters Patent No. 434,016, dated August 12, 1890.

Application filed October 22, 1889. Serial No. 327,619. (No specimen.)

*To all whom it may concern:*

Be it known that I, HARRIETT B. DEVLAN, a citizen of the United States, residing at Jersey City, in the county of Hudson and State of New Jersey, have invented new and useful Improvements in Anti-Friction Material for Journal-Bearings, of which the following is a specification.

The object of my invention is to provide an improved anti-friction and heat-resisting material for journal bearings or boxes, whereby overheating of journals and journal-bearings can be prevented; and to this end the invention consists in an anti-friction material composed of pulped bamboo fibers, or paper-pulp and pulped bamboo fibers impregnated with pulverized plumbago, or graphite, soapstone, or steatite and asbestos, and a sizing, such as silicate of soda, as hereinafter set forth.

In carrying my invention into effect I make a pulp from bamboo fibers in the usual manner in which paper-pulp is prepared, and into this bamboo pulp I put about twenty-five per cent. of pulverized plumbago, (graphite), or about the same quantity of pulverized soapstone, (steatite), or any fine earthy matter. I also place in the mixture about twenty-five per cent. of asbestos. After these materials are thoroughly mixed I add about twenty-five per cent. of silicate of soda, or potash, or any other suitable sizing. In some cases I may use paper-pulp in conjunction with pulped bamboo fibers. The pulp thus prepared is passed over rollers in the same manner as in the operation of making paper or pasteboard, and the fibrous sheets thus produced are compressed and calendered by passing them between suitable rollers.

This improved fibrous anti-friction material is prepared for use by cutting the sheets into blocks or pieces of appropriate shape and dimensions to serve as linings or coverings for journal bearings or boxes, being secured thereto in any convenient or proper manner. When worn, this anti-friction material can be readily removed and replaced by fresh material of the same character at but slight expense.

I have found by actual experiment and use that bamboo fibers possess great heat-resisting qualities and tend to cool a journal or axle more effectually than any other fibrous material of which I am aware. Asbestos contributes to the same result, but is not essential to the compound contemplated by my invention, though I prefer to use it in conjunction with the other substances above named. The mineral and earthy substances named also serve to give body to the anti-friction compound, besides aiding it to resist the action of heat and thus preventing undue heating of the axle or journal. The plumbago and steatite contribute also a lubricant quality to the compound and render it particularly useful as an anti-friction covering or lining for journal bearings or boxes.

The proportions of the several ingredients herein named give good results; but I do not wish to be understood as confining myself to any specific proportions, since they may be varied to suit various conditions.

The most important ingredient of my improved anti-friction material is the pulp prepared from bamboo fibers, which I have found possesses the quality of resisting heat to a marked degree, and is thus extremely useful in a compound of this character.

What I claim as my invention is—

1. A packing for journal-boxes, consisting of bamboo fiber, a sizing, such as silicate of soda, and a mineral substance, such as plumbago, substantially as described.

2. A packing for journal-boxes, consisting of bamboo fiber, a sizing, such as silicate of soda, plumbago, and asbestos, substantially as described.

3. A packing for journal-boxes, consisting of bamboo fiber, paper-pulp, asbestos, plumbago, and a sizing, such as silicate of soda, substantially as described.

In testimony whereof I have affixed my signature in presence of two witnesses.

HARRIETT B. DEVLAN.

Witnesses:

WILLIAM J. ROUGET,  
FRANK NOLAN.